

## UNITED STATES PATENT OFFICE

2,281,648

PROCESS OF PRODUCING A CHLORINATED  
MINERAL OIL AND THE OIL RESULTING  
THEREFROMEverett R. Wiles, Barnsdall, Okla., assignor to  
Barco Oil Company, Tulsa, Okla., a corpora-  
tion of DelawareNo Drawing. Application January 2, 1936,  
Serial No. 57,251

6 Claims. (Cl. 260—654)

My invention relates to lubricating oils and more particularly to a chlorinating process for producing an oil which is suitable particularly as an addition agent to an oil for lubricating machinery operating under conditions imposing excessive lubricating requirements such as at unusually high speeds and high bearing pressures.

Mineral oil lubricants have been developed to a high degree of efficiency as lubricating agents but it is now apparent that certain types of machinery have come into use which are difficult to lubricate with any known refined mineral oil in its natural form, that is, without the addition thereto of other materials. For example, the use of metals of greater strength in designing motor cars has permitted the use of greatly increased pressures between various metal parts. These pressures are now commonly so great under certain operating conditions that an ordinary oil film between the surfaces will break down or rupture allowing metal to metal contact. Various suggestions have been made for producing a lubricating oil having film characteristics suitable to meet these conditions usually present in machinery employing high speed and high bearing pressures. Such suggestions include the use of fatty oils and acids, the incorporation of elementary and combined sulphur, the use of various metallic soaps, either suspended or in solution in mineral oils, and the use of certain chlorine compounds added to the oil. Nearly all of these materials present some practical difficulty such as insolubility, abrasiveness and corrosiveness and furthermore their lubricative action under conditions of stress is not always satisfactory.

Chlorine compounds are in some respects very desirable materials for incorporation in the mineral oils to improve their lubricating characteristics when the oils are used under extreme conditions. While these chlorine compounds are of value in serving to protect the machinery by providing better lubrication, particularly under high pressure conditions, the use of such compounds is ordinarily limited mainly by two factors. First, the chlorination compounds are almost invariably corrosive or become corrosive on standing, and in such condition their use is absolutely prohibited. Secondly, the chlorine compounds, particularly chlorine treated mineral oils are very apt to undergo a reaction in use with the formation of gums and resins. This latter characteristic, unless controlled, is quite detrimental from the lubrication standpoint because of the fact that the gums which settle out are

deposited in the gears and other movable parts of the machinery and interfere with its operation and cause these parts to deteriorate because of lack of adequate lubrication. The chlorinating process of our invention is carried out in such a manner that these deleterious gums and resins are eliminated from the oil before it is used.

I have found that the undesirable corrosive characteristics of the chlorinated mineral oils result mainly from the instability of certain of the compounds formed during chlorination, and that certain other compounds are formed during this period with a stability making them desirable for use as base material for extra pressure lubricants.

It is very important that the stability of the chlorine compounds be exactly gauged, that is, they must be stable enough to stand storage without change and yet the stability must not be so great as to prohibit change under conditions which would give film rupture of the carrier oil. Under the latter conditions the chlorine compounds should become sufficiently active to provide the necessary lubrication not produced by the carrier oil. In other words, the material which is added to the ordinary lubricating oil to give it the necessary extra lubricating qualities must of itself be a good lubricant, and must be stable under certain conditions, non-corrosive and non-gumming. It should be present preferably in only small quantities and should even then not develop characteristics other than those of a normally good lubricant under ordinary conditions of speed and load. Under extraordinary conditions, however, such as excessive load and high temperature which cause the ordinary lubricating oil to break down with resultant film rupture and failure of the bearing, this added material should become operative and supply the additional necessary lubrication or other effect to protect the bearing. The chlorinated oils of our invention possess these desirable characteristics.

One of the objects of my invention is to provide an improved lubricating oil which is capable of adequately lubricating machinery operating at extremely high speeds and pressures and under what are at present considered extreme lubricating conditions.

Another object is to provide an improved process for chlorinating a mineral oil such that the chlorinated oil will be substantially free of corrosive and gum-forming characteristics.

Still another object of the invention is to provide an oil which when added to ordinary lubri-

cating oil will possess only normal lubricating qualities under ordinary operative conditions but when subjected to excessive high speed and pressure conditions, under which ordinary lubricating oil will fail and cause deterioration of the machinery, will provide sufficient extraordinary lubrication or other effect to prevent such deterioration.

In accordance with my invention I have developed a process for treating mineral oil in such a manner that it will possess all of the desired characteristics described above, so that when it is added in desired amounts to an ordinary lubricating oil the resulting mixture will fulfill all of the requirements for lubrication of machinery operating under normal conditions and also under unusually high speed and high pressure conditions. In general my process comprises, as the first step, passing chlorine into a suitable neutral mineral oil while the latter is constantly agitated and maintained at a relatively low temperature, preferably below 50° F. Corrosion-resisting materials are used while mixing and agitating the oil to prevent corrosive effects which would otherwise be produced by the free chlorine and hydrochloric acid formed during chlorination. A small amount of air or other carrier gas is preferably blown through the oil during chlorination. This air serves the purpose of sweeping out free chlorine and gaseous hydrochloric acid generated during the chlorinating process, the oil having a tendency to foam when it approaches saturation with hydrochloric gas. A slight negative pressure instead of blowing with air might also be used to prevent foaming.

The hydrochloric acid gas carried away by the air is recovered by condensation or absorption methods to produce a high grade of technical hydrochloric acid of between 25 to 30% concentration which constitutes a valuable and easily recovered by-product of this process. Chlorine used in the process may be recovered as 30% water solution of hydrochloric acid to the extent of 75% or more of such solution of hydrochloric acid on the basis of the original chlorine used.

The chlorination of the oil is carried to the desired point, which may be determined by measurement of the specific gravity of the oil at different times during the chlorination process. The specific gravity, of course, increases as the chlorination proceeds and the further the chlorination proceeds the more effective is the final material as a pressure-carrying lubricant.

In certain cases it may be desirable to chlorinate only to approximately 1.0 specific gravity or if desired chlorination may be carried out until a specific gravity of 1.2 or greater results. As a general rule the further chlorination proceeds the more effective the final material as a pressure carrying lubricant. By this is meant that not only less of the base material is necessary to produce a certain result, but actually less total chlorine in the final blended material is needed, or in other words, the chlorine appears to act more efficiently.

I have also found that chlorination carried out below 50° F., and preferably at about 35° F., gives a more desirable product than one produced by chlorinating above 50° F. For example, a lubricating oil containing 5% of a base of 12% chlorine content, chlorinated below 50° F., exhibited extreme pressure characteristics far in excess of an oil containing an equivalent base chlorinated above 50° F.

When chlorination is complete the cold chlorinated oil is mixed with alkali for example 30-35% by volume of a solution of 30-40° Bé. gravity caustic soda. This alkali causes a substantial neutralization of the acids contained in the oil and also serves to remove the excess chlorine and HCl present. Next, the chlorinated oil and alkali is agitated and heated to approximately 200° F., which temperature is maintained for quite a number of hours, depending upon the type of oil being used, but usually sixty to seventy hours.

This part of the process is known as the "cooking out" of the oil, and has three main objectives.

15 First, the complete neutralization of the oil; second, production of exactly the proper stability of the oil, and third, removal of compounds that would form gums when the oil is used. By this 20 operation the combined chlorine may be rearranged and the molecule stabilized and the gum-forming compounds condensed and polymerized to form insoluble resins and gums which are then removed by suitable means, for example, centrifuging or filtering or simple decanting. The 25 stabilizing of the oil is apparently one of rearrangement rather than elimination of the chlorine for there is a loss of chlorine of usually only about 1% as a result of the operation on an oil basis.

The oil processed in the manner described 30 above is allowed to settle and is clarified by filtering or other means and is then ready for use. In use this oil which we call the base oil, is incorporated into any desirable lubricating oil in the proper amounts to give the pressure-carrying 35 properties desired. This may be determined by the use of any standard type testing apparatus, such as the Almen, Timken, or Floyd machines. The amounts of this base oil to be added to the ordinary lubricating oil may vary from 1/4 of 1% 40 to 20%, although normally the amount is about 5% by volume of the type of 1.00 sp. gr. chlorination.

In one specific embodiment of the process of my invention, the mineral oil which I chlorinated 45 was a light neutral oil having a Saybolt Universal viscosity of approximately 100 seconds at 100° F. While any other similar starting material would do as well from the standpoint of extra pressure lubrication, I found that this oil is suitable from 50 the standpoint of practical operation and manufacture. The oil, which had originally a specific gravity of .89 was run into a wooden tank and chlorine introduced into the oil at the bottom of the tank close to a mechanical agitator. The 55 temperature of the oil was maintained by means of cooling coils between 30° F. and 50° F. Chlorination was continued until the oil attained a specific gravity of 1.15. Such an oil has a chlorine content of approximately 25%. Approximately 1% of this product was found to be equivalent to 5% of a 1.00 sp. gr. (12% Cl) product on an Almen machine test.

Phosphor bronze was found satisfactory as a 60 corrosive-resisting material for the agitator. Air was admitted during the chlorination process to carry off, through a wooden flume the excess chlorine and hydrochloric acid gas generated during chlorination, which elimination tends to diminish the tendency towards foaming of the oil during chlorination.

After chlorination the cold chlorinated oil was 65 mixed with approximately 35%, by volume, of a 35° Bé., gravity sodium hydroxide solution. The mixture of chlorinated oil and sodium hydroxide 70 was then heated to 200° F. and "cooked" for ap-

proximately 65 hours, during which time constant agitation of the mixture was maintained. After this "cooking" process was completed, that is, after products of the desired stability were obtained, there having been a progressive rise in temperature at which the chlorine compounds break down, the oil was filtered and the filtrate mixed with an ordinary lubricating oil. The stability of the oil may be determined at intervals by withdrawing a sample, subjecting it to slowly increased heating, and determining that temperature at intervals chlorine is first liberated indicating the upper stabilized limit. The oil may be made stable to temperature of about 350° F., although the break down point may be raised or lowered, for example to 400° F., or to 250° F., by the stabilizing treatment to produce one suitable for a specific use.

I found that the resulting chlorinated oil from this illustrative treatment had been so modified or rearranged with particular regard to the chlorine compounds that they were in a stable form when subjected to ordinary conditions of lubrication but were sufficiently unstable at abnormal conditions of lubrication to become effective in facilitating lubrication and preventing metal to metal contact. Thus, they provide excellent lubrication under normal as well as high speed, high temperature, and high pressure conditions necessary for operation in many modern types of machinery.

While I do not wish to limit myself to any theory, I believe that the unusually good lubricating qualities of the oil produced by my inventive process may result from the fact that the especially prepared base oil which is added to the ordinary lubricating oil remains practically inert under ordinary operating conditions but under extraordinary conditions, such as those of high temperature and high pressures, this base oil becomes operative and breaks down to some slight extent, locally and at points of high temperature, liberating chlorine which combines with the material of the bearing. This may form a protective coat which is highly retentive for lubricating oil and thus assist in preventing the failure of the bearings and associated parts. As soon as the extraordinary condition period has passed the base oil again assumes its function of a normal lubricant without further liberation of chlorine.

It is to be understood that my invention is not limited to the specific processes described above by way of example, but is susceptible to various changes and modifications, the scope of which is limited only by the following claims.

What I claim is:

1. The process of preparing a mineral oil suitable for lubricating machinery under normal operating conditions and also under conditions of extremely high temperature and pressure, com-

prising chlorinating the oil at a temperature less than 50° F., neutralizing the acids in the chlorinated oil by mixing the oil with an alkali solution, stabilizing the oil by heating it with alkali until practically all of the gums and resins settle out, and removing said gums and resins from the oil.

2. A process for chlorinating mineral oils to increase their lubricating efficiency which consists in passing chlorine into a neutral mineral oil during constant agitation of the oil, maintaining the oil at a temperature between 25° F. and 50° F., blowing air through the oil during agitation to remove the excess chlorine and hydrochloric acid gas formed during the chlorinating treatment and treating the resulting chlorinated oil with an alkali by heating for a number of hours.

3. The process for producing an extra pressure lubricant consisting of chlorinating a mineral oil, cooling the oil during chlorination to maintain the temperature below 50° F., neutralizing the oil with an alkaline substance, heating the oil and alkaline substance for several hours at approximately 200° F. to establish the desired stability of the oil and to condense and polymerize the gums and resins filtering the stabilized oil, and adding the filtered oil to an ordinary lubricating oil in such amounts that the filtered oil constitutes from approximately  $\frac{1}{4}$  of 1% to 20% of the total weight of the oil.

4. A stabilized chlorinated neutral hydrocarbon lubricant suitable for use as a high pressure lubricating base and produced by chlorinating a mineral oil while maintaining the temperature of the oil below 50° F., heating the oil for a prolonged period in the presence of an alkaline substance to a temperature approximately of 200° F., and removing polymerized gums and resins.

5. A stabilized chlorinated neutral hydrocarbon lubricant suitable for use as a high pressure lubricating base and produced by chlorinating a mineral oil while maintaining the temperature of the oil below 50° F., heating the oil for a period of about sixty to seventy hours in the presence of an alkaline substance to a temperature of approximately 200° F. and removing polymerized gums and resins.

6. A process for producing a lubricating oil consisting of chlorinating a mineral oil, cooling the oil during chlorination to maintain the temperature below 50° F., neutralizing the oil with an alkali, heating the oil and alkali for a period of about sixty to seventy hours at approximately 200° F. to condense and polymerize the gums and resins in the oil and to establish the desired stability of the oil, and filtering the stabilized oil.

EVERETT R. WILES.